

## UNITED STATES PATENT OFFICE

2,193,023

## PHOTOGRAPHIC REVERSAL PROCESS

Ralph M. Evans and Wesley T. Hanson, Jr.,  
Rochester, N. Y., assignors to Eastman Kodak  
Company, Rochester, N. Y., a corporation of  
New Jersey

No Drawing. Application April 6, 1938,  
Serial No. 200,507

6 Claims. (CL. 95—88)

This invention relates to developing photographic images and particularly to a method for producing positive images by reversal.

Photographic reversal images are produced in two general ways. In each of these the sensitive layer is exposed to light and the original latent image is developed to a negative. The negative silver image produced in this way is then removed without destroying the sensitivity of the unexposed silver halide. This is usually done by means of a bath of potassium permanganate and sulfuric acid. After removal of the negative silver image in this way, the sensitive layer may be either exposed to light or chemically fogged without exposure to light, to produce a latent image which may then be developed in the usual way to produce a positive reversal image.

It is an object of the present invention to simplify this reversal process by providing a means for omitting one of the customary steps. A further object is to provide a method for producing a black and white reversal image in a silver halide layer without removal of the negative silver image prior to the final fixing step. Other objects will appear from the following description of our invention.

These objects are accomplished by carrying out the reversal development in a coupler developer which produces both a silver image and also a dye image which protects the silver image so that it is not removed in later oxidizing baths, such as ferricyanide and hypo.

In carrying out our process the sensitive layer is first exposed, either to an object or under a transparency of an image, and is developed to a negative silver image in an ordinary developer, such as a customary metal-hydroquinone developer. The layer is then thoroughly washed in water and is exposed to the desired extent without removal of the negative silver image. This exposure may be made either from the emulsion side or through the support in the case of a film or plate. The layer is then developed to the required density in a coupler developer which forms a positive silver image and a dye image simultaneously in the layer. The coupler compound must be one which produces a dye of substantially neutral grey density or which protects the positive silver image in such a way that it is not removed in subsequent baths of the process. The layer is then fixed in a solution, such as potassium ferricyanide and hypo, which removes either the negative silver image or both the negative and positive silver images without affecting the positive dye image. The positive

dye or dye and silver image remaining after this treatment is substantially neutral grey in color and is found to be a satisfactory image in either transparencies, such as films or plates, or in photographic paper.

A coupler developer which we have found to be satisfactory for producing the reversal image is one using a p-phenylenediamine developing agent and p-benzyl phenol as the coupling compound. Other coupling compounds which produce substantial neutral grey dye images may also be used.

The following examples, which are illustrative only, indicate developing solutions which may be used for the reversal development, according to our invention:

## Example I

|                             |       |    |
|-----------------------------|-------|----|
| Diethyl p-phenylene diamine | grams | 3  |
| Sodium carbonate            | do    | 30 |
| Sodium sulfite              | do    | 6  |
| p-Benzyl phenol             | do    | 3  |
| Sodium hydroxide            | do    | 5  |
| Water to                    | liter | 1  |

## Example II

|                                               |       |    |
|-----------------------------------------------|-------|----|
| 2-amino-5-diethyl amino toluene hydrochloride | grams | 3  |
| Sodium sulfite                                | do    | 6  |
| Sodium carbonate                              | do    | 45 |
| Potassium bromide                             | do    | 1  |
| Potassium thiocyanate                         | do    | 1  |
| p-Benzyl phenol                               | do    | 4  |
| Sodium hydroxide                              | do    | 5  |
| Water to                                      | liter | 1  |

It is to be understood that we may use any of the usual p-phenylene diamine coupler developers other than those referred to above, such as dimethyl p-phenylene diamine, or any other p-phenylene diamine developer containing a primary amino group. The developing solution may also contain other well known ingredients and the proportions of the various developer constituents may be varied over wide ranges.

Other well known expedients of photographic reversal processes may be used in conjunction with our reversal development. For example, the light exposure prior to the reversal development may be controlled to produce the desired density in the final image. If the original exposure is too great, a longer second exposure can be given and vice versa so that a constant developing time will afford equally good results. The process of controlling the second exposure in our process is somewhat different from that used in

the customary reversal processes in which the silver is removed before the second exposure so that an over-exposed film has a high transmission and an unexposed film has a lower transmission. In the present process an overexposed negative will have a very low transmission and an unexposed negative will have a high transmission, and a suitable exposure control method must be used. This method of controlling the density of the final image in a color development reversal process is described in Seymour U. S. Patent No. 1,939,231, granted December 12, 1933.

The action of p-benzyl phenol in a coupler developer is somewhat different than that of the majority of coupler compounds in that it prevents the removal of the metallic silver by treatment in the usual oxidizing baths. The final image is, therefore, a combined silver and dye image which is substantially neutral grey in color and which is highly satisfactory for the production of black and white photographic images. Although we do not wish to be limited to any particular explanation of the reason for this action, we believe that the dye formed by union of the p-benzyl phenol with the oxidation product of p-phenylene diamine developing agent protects the metallic silver image in some manner such as by formation of a protective coating of the dye around the silver image, so that the oxidizing baths are not able to attack the silver.

It is to be understood that numerous other modifications and equivalents are possible in our process and that our invention is to be limited only by the scope of the appended claims.

What we claim is:

1. The method of forming a photographic reversal image having a substantially neutral grey color which comprises exposing a gelatino-silver halide layer to a light image to form a negative latent image therein and developing said latent image to metallic silver, exposing the layer to a uniform light source, without removing the negative silver image from the layer, developing the layer in a developing solution containing a p-phenylene diamine developing agent and a p-benzyl phenol coupler compound to form a positive image in the layer and removing the metallic silver negative image from the layer.

2. The method of forming a photographic reversal image having a substantially neutral grey color which comprises exposing a gelatino-silver halide layer to a light image to form a negative latent image therein and developing said latent image to metallic silver, exposing the layer to a uniform light source, without removing the negative silver image from the layer, developing the layer in a developing solution containing a p-phenylene diamine developing agent and a p-benzyl phenol coupler compound to form a positive image in the layer and fixing the layer in a ferricyanide and hypo bath. 5

3. In the method of producing a black and white photographic image by reversal, the step 15 which comprises developing the reversal image in a coupler developer containing a p-phenylene diamine developing agent and a p-benzyl phenol coupler compound.

4. In the method of producing a black and white photographic image by reversal, the steps 20 which comprise developing a negative metallic silver image in the layer and without removal of the metallic silver image, developing a reversal image in the layer in a coupler developer containing a p-phenylene diamine developing agent and a p-benzyl phenol coupler compound. 25

5. In the method of producing a black and white photographic image by reversal, the steps 30 which comprise developing a metallic silver negative image in the layer and without removal of the negative image, developing in the layer a reversal image in a coupler developer comprising a diethyl p-phenylene diamine developer and a p-benzyl phenol in substantially equal amounts. 35

6. In the method of producing a black and white photographic image by reversal, the steps 40 which comprise developing a metallic silver negative in the layer and without removal of the negative image, developing in the layer a reversal image in a coupler developer comprising a diethyl p-phenylene diamine developer and p-benzyl phenol in substantially equal amounts, and removing the metallic silver negative image from the layer. 45

RALPH M. EVANS.  
WESLEY T. HANSON, JR.